



US012397396B2

(12) **United States Patent**  
**Yamaguchi et al.**

(10) **Patent No.:** **US 12,397,396 B2**  
(45) **Date of Patent:** **Aug. 26, 2025**

(54) **METHOD FOR MANUFACTURING POROUS METAL BONDED GRINDSTONE, AND METHOD FOR MANUFACTURING POROUS METAL BONDED WHEEL**

(71) Applicant: **NORITAKE CO., LIMITED**, Nagoya (JP)

(72) Inventors: **Masaru Yamaguchi**, Nagoya (JP); **Daiki Furuno**, Nagoya (JP)

(73) Assignee: **NORITAKE CO., LIMITED**, Nagoya (JP)

(\*) Notice: Subject to any disclaimer, the term of this patent is extended or adjusted under 35 U.S.C. 154(b) by 324 days.

(21) Appl. No.: **18/251,644**

(22) PCT Filed: **Oct. 14, 2021**

(86) PCT No.: **PCT/JP2021/038076**

§ 371 (c)(1),  
(2) Date: **May 3, 2023**

(87) PCT Pub. No.: **WO2022/102335**

PCT Pub. Date: **May 19, 2022**

(65) **Prior Publication Data**

US 2023/0405764 A1 Dec. 21, 2023

(30) **Foreign Application Priority Data**

Nov. 10, 2020 (JP) ..... 2020-187173

(51) **Int. Cl.**  
**B24D 3/10** (2006.01)

(52) **U.S. Cl.**  
CPC ..... **B24D 3/10** (2013.01)

(58) **Field of Classification Search**  
CPC ..... B24D 3/10; B24D 3/06  
See application file for complete search history.

(56) **References Cited**

U.S. PATENT DOCUMENTS

4,917,960 A 4/1990 Hornberger  
2003/0097800 A1\* 5/2003 Ramanath ..... C09K 3/1409  
51/309

FOREIGN PATENT DOCUMENTS

CN 101450463 A 6/2009  
CN 101528954 A 9/2009

(Continued)

OTHER PUBLICATIONS

The International Preliminary Report on Patentability for the corresponding international application No. PCT/JP2021/038076 issued May 16, 2023, which includes English translation of Written Opinion of the International Searching Authority for the corresponding international application No. PCT/JP2021/038076 mailed Dec. 7, 2021.

(Continued)

*Primary Examiner* — Pegah Parvini

(74) *Attorney, Agent, or Firm* — Muncy, Geissler, Olds & Lowe, P.C.

(57) **ABSTRACT**

A method for manufacturing a porous metal bonded grindstone with which it is possible to arbitrarily adjust a porosity from a low porosity to a high porosity is provided. This method is intended for manufacturing the porous metal bonded grindstone and comprises: a molding step (P1) for obtaining an unfired molded body including abrasive grains, metal powder, and a pore forming material; a solute removing step (P2) for bringing vapor of a solvent having solubility with respect to the pore forming material into contact with the unfired molded body to remove the pore forming material and to obtain an unfired molded body having pores; and a firing step (P3) for firing the unfired molded body having pores.

**7 Claims, 3 Drawing Sheets**



(56)

**References Cited**

FOREIGN PATENT DOCUMENTS

|    |               |    |   |         |       |              |
|----|---------------|----|---|---------|-------|--------------|
| JP | 63-212059     | A  | * | 9/1988  | ..... | B22D 19/00   |
| JP | S63212059     | A  |   | 9/1988  |       |              |
| JP | H08-81703     | A  |   | 3/1996  |       |              |
| JP | 2001088035    | A  |   | 4/2001  |       |              |
| JP | 2005525242    | A  |   | 8/2005  |       |              |
| JP | 2008030194    | A  |   | 2/2008  |       |              |
| JP | 2010540261    | A  |   | 12/2010 |       |              |
| JP | 2019104079    | A  |   | 6/2019  |       |              |
| WO | WO-2016081302 | A1 | * | 5/2016  | ..... | B24D 18/0009 |

OTHER PUBLICATIONS

The First Office Action of the corresponding CN application No. 202180075016.7 mailed May 30, 2025 and English translation thereof.

\* cited by examiner

[Fig. 1]



[Fig. 2]



[Fig. 3]



[Fig. 4]



[Fig. 5]



[Fig. 6]



**METHOD FOR MANUFACTURING POROUS  
METAL BONDED GRINDSTONE, AND  
METHOD FOR MANUFACTURING POROUS  
METAL BONDED WHEEL**

TECHNICAL FIELD

The present invention relates to a method for manufacturing a porous metal bonded grindstone. The present invention also relates to a method for manufacturing a porous metal bonded wheel.

BACKGROUND ART

Conventionally, a vitrified bonded grindstone has been used as a grindstone suitable for grinding high-hardness fragile materials by a stable grinding capability with high efficiency and a long-life duration. Conventionally, there has not been much demand for grinding high-hardness fragile materials and it was sufficient to perform this by taking time for the grinding. However, as the power device market and LED market expand, the demand for the processing with high efficiency and a long-life duration has increased for such grinding, for the purpose of productivity improvement and processing cost reduction. Therefore, a grindstone for achieving these purposes is required.

In a high-efficiency and high-precision processing field and in a processing field called super finishing for the above high-hardness fragile materials, porous metal bonded grindstones are sometimes used as a tool which is superior in having a long-life duration. As methods for manufacturing the porous metal bonded grindstones, there have been known, for example, a method for forming pores by adding closed-cell cellular materials such as hollow fine particles, a method for forming pores by adding organic media and burning-through by firing, and a method for forming pores by adding salt and eluting it in a solvent after firing.

For example, Patent Literature 1 discloses a porous grindstone characterized in that abrasive grains and inorganic hollow fine particles disperse in a metal binder or a vitreous binder. Patent Literature 1 also discloses that a mixture powder obtained by mixing the abrasive grains, the hollow fine particles, and the powder of the metal binder is heated and cooled after melting the metal binder, so that the porous grindstones can be manufactured.

Patent Literature 2 discloses a composite material for grinding a workpiece composed of a hard material to achieve desired surface finishing, the composite material containing specific abrasive grains, a specific metal binder, and porous portions at a specific ratio, as well as a method for manufacturing the same. Patent Literature 2 also describes immersing an abrasive article in a solvent to leach out the dispersoid, so that interconnected pores are left in the abrasive article.

Patent Literature 3 discloses a method for manufacturing an abrasive article with interconnected pores of at least 50 vol %, the method comprising the steps of: (a) admixing a mixture containing abrasive grains of about 0.5 to about 25 vol %, a binder of about 19.5 to about 49.5 vol %, and dispersoid particles of about 50 to about 80 vol %; (b) pressing the mixture into a composite material filled with abrasive materials; (c) performing thermal processing on the composite material; and (d) immersing the composite material in a solvent in which the dispersoid particles are dissolved over a fixed time suitable for substantially dissolving

all of the dispersoid particles, wherein the abrasive grains and the binder are substantially insoluble with respect to the solvent.

5 CITATION LIST

Patent Literature

10 Patent Literature 1: JP 2001-88035 A  
Patent Literature 2: JP 5314030 B2  
Patent Literature 3: JP 2008-30194 A

15 SUMMARY OF INVENTION

Technical Problem

20 As in Patent Literature 1, in the method for forming the pores by using the closed-cell cellular materials such as hollow fine particles, porosity can be adjusted in accordance with the amount of addition of the closed-cell cellular materials. However, the contours of the pores remain as unnecessary residues and therefore, in case of using the 25 grindstone as the tool, the residues contact with the workpiece at the time of processing, so that there is concern about grinding burning accompanied by increase in resistance and deterioration of processing precision.

25 According to a method for causing a pore forming material such as a dispersoid to be eluted into a solvent in order to form the pores, no unnecessary residues such as the contours of the closed-cell cellular materials remain. Further, as shown in FIG. 6, according to the conventional 30 method for manufacturing a porous metal bonded grindstone, a solute removing step is carried out after a firing step. After undergoing the firing step, a fired body in which the abrasive grains are strongly adhered to a metal bond can be 35 obtained, it is possible to suppress the strength of the metal bond and the adhesion force of the abrasive grains from lowering even if the fired body is immersed in the solvent, and the pore forming material can be eluted. However, since the metal bond is strongly fired and hardened, the pore forming materials need to interconnect with each other in 40 order to allow the solvent to penetrate. If the ratio of the pore forming materials in the fired body is too low, there occurs a portion in which the pore forming materials do not 45 interconnect with each other, so that the solvent cannot penetrate, thus making it difficult to elute the pore forming materials. The pores need to interconnect with each other in order to dissipate all the dispersoids. For example, according 50 to the methods of Patent Literatures 2 and 3, the dispersoids of at least 40 vol % need to be added. However, in case of using, as the tool, a grindstone with the porosity of at least 55 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770

out that the following invention conforms to the above object and have conceived the present invention.

Namely, the present invention relates to the following invention.

<1> A method for manufacturing a porous metal bonded grindstone, comprising: a molding step for obtaining an unfired molded body including abrasive grains, metal powder and a pore forming material; a solute removing step for bringing vapor of a solvent having solubility with respect to the pore forming material into contact with the unfired molded body to remove the pore forming material and to obtain an unfired molded body having pores; and a firing step for firing the unfired molded body having pores.

<2> The method for manufacturing a porous metal bonded grindstone according to above <1>, wherein a volume ratio of the pore forming material to the unfired molded body is from 5 to 90 vol %.

<3> The method for manufacturing a porous metal bonded grindstone according to above <1> or <2>, wherein an average particle size of the pore forming material is from 5 to 250  $\mu\text{m}$ .

<4> The method for manufacturing a porous metal bonded grindstone according to any of above <1> to <3>, wherein the solvent contains at least one selected from the group consisting of water, alcohol, and acetone.

<5> The method for manufacturing a porous metal bonded grindstone according to any of above <1> to <4>, wherein the solvent contains water and the pore forming material is a water-soluble compound.

<6> The method for manufacturing a porous metal bonded grindstone according to above <5>, wherein the pore forming material is a water-soluble inorganic salt.

<7> A method for manufacturing a porous metal bonded wheel, comprising the steps of: bonding, to a base metal, a porous metal bonded grindstone manufactured in accordance with the method for manufacturing the porous metal bonded grindstone according to any of above <1> to <4>; and finishing the porous metal bonded grindstone bonded to the base metal by using a dresser.

#### Advantageous Effects of Invention

According to the present invention, the method for manufacturing the porous metal bonded grindstone which uses pore forming materials which enable the elution by the solvent and with which it is possible to adjust the porosity arbitrarily from a low porosity to a high porosity is provided. In this manner, the porous metal bonded grindstone in which the influence of the unnecessary residue such as the contour of the closed-cell cellular material is suppressed, can be obtained with a desired porosity.

Further, the method for manufacturing the porous metal bonded wheel comprising the porous metal bonded grindstone having an arbitrary porosity from a low porosity to a high porosity is provided.

#### BRIEF DESCRIPTION OF DRAWINGS

FIG. 1 is a process chart of the method for manufacturing the porous metal bonded grindstone in the present invention.

FIG. 2 is a partial cross sectional schematic drawing showing the grindstone manufactured in accordance with the method for manufacturing the porous metal bonded grindstone in the present invention.

FIG. 3 is a drawing for explaining a state of the porous metal bonded grindstone of the present invention at the time of grinding.

FIG. 4 is a process chart of the method for manufacturing the porous metal bonded wheel in the present invention.

FIG. 5 is a perspective view showing one example of a porous metal bonded grindstone manufactured in accordance with the method for manufacturing the porous metal bonded wheel in the present invention.

FIG. 6 is a process chart of the method for manufacturing the conventional porous metal bonded grindstone.

#### DESCRIPTION OF EMBODIMENTS

Hereinafter, embodiments of the present invention will be explained in detail. The following explanation about the components relates to one example (representative example) 15 of an aspect of the present invention and is not limited to the following contents as far as the gist of the present invention is not changed. When the expression “[ . . . ] to [ . . . ]” is used in the present specification, it is used as the expression including the numerical values or the physical property 20 values before and after this expression.

##### <Method for Manufacturing Porous Metal Bonded Grindstone in the Present Invention>

The present invention relates to a method for manufacturing a porous metal bonded grindstone, comprising: a molding step for obtaining an unfired molded body including abrasive grains, metal powder and a pore forming material; a solute removing step for bringing vapor of a solvent having solubility with respect to the pore forming material into contact with the unfired molded body to 25 remove the pore forming material and to obtain an unfired molded body having pores; and a firing step for firing the unfired molded body having pores (hereinafter sometimes referred to as “the method for manufacturing the grindstone in the present invention”).

The method for manufacturing the grindstone in the present invention is characterized in that the pore forming material is removed while the molded body is in the unfired state and the vapor is used for removing the pore forming material. As described above, the pore forming material is 40 removed while the molded body is in the unfired state (namely, the solute removing step is carried out before the firing step), so that the molded body is not strongly fired and hardened, and therefore the vapor of the solvent easily penetrates into its inside. Therefore, even if the amount of

45 the pore forming materials is small, the vapor of the solvent can penetrate into the inside of the molded body and the pore forming material can be sufficiently eluted. Further, the molded body is made to contact with the vapor of the solvent without immersing the molded body in the solvent, so that the vapor easily penetrates further into the interior of the molded body. Further, since the unfired molded body has a 50 low shape stability, the shape is likely to dissolve when the unfired molded body is immersed in the solvent. Meanwhile, according to the method for manufacturing the grindstone in 55 the present invention, the unfired molded body is made to contact with the vapor of the solvent, so that the shape of the molded body is difficult to dissolve even if it is unfired. By firing the thus obtained unfired molded body having pores formed therein, the metal powder is melted and fired while the pores remain maintained as they are, so that it is possible to manufacture the porous metal bonded grindstone with the pore forming material sufficiently removed in spite of the low porosity.

FIG. 1 is a process chart of the method for manufacturing 60 the porous metal bonded grindstone in the present invention. Hereinafter, each step will be explained based on FIG. 1. [Molding Step (P1)]

The molding step is a step for obtaining the unfired molded body including the abrasive grains, the metal powder, and the pore forming material.

(Abrasive Grains)

As the abrasive grains, diamonds, etc. can be used. The average particle size of the abrasive grains can be appropriately selected based on the type of a material to be ground, etc. In case of grinding high-hardness fragile materials such as a silicon carbide and a sapphire, the abrasive grains deeply eat into the high-hardness fragile material and the damage reaches its interior, so that the processing time becomes long during the next step. When the average particle size of the abrasive grains is too large, the abrasive grains tend to eat deeply into the material to be ground, thereby increasing the damage to the material to be ground. Meanwhile, if the average particle size of the abrasive grains is too small, the abrasive grains tend not to eat into the material to be ground, so that it is difficult to carry out the processing. Therefore, the average particle size of the abrasive grains is desirably from 4 to 55  $\mu\text{m}$ . For example, in case of grinding a sapphire wafer, the average particle size can be from 12 to 55  $\mu\text{m}$ . In case of grinding a silicon carbide (SiC) wafer which is more difficult to process, the average particle size is desirably from 4 to 20  $\mu\text{m}$ .

In the present application, the average particle size is a median size of particle size distribution measured by a particle size distribution measuring instrument (laser refraction scattering method). The median size is a volume-based D50 value measured by using a laser diffraction/scattering particle size distribution measuring instrument (LA-960) by HORIBA, Ltd. in accordance with the measurement method conforming to JIS Z 8825:2013.

(Metal Powder)

As the metal powder, at least one selected from the group consisting of copper, tin, cobalt, iron, nickel, tungsten, silver, zinc, aluminum, titanium, zirconium, and an alloy thereof can be used. Generally, the metal powder preferably contains a mixture of copper and tin. For example, as for grinding the high-hardness fragile material, a composition preferably contains copper of about 30 mass % to about 70 mass % and tin of about 30 mass % to about 70 mass %.

(Pore Forming Material)

For the pore forming material, arbitrary solute particles which can easily dissolve in the solvent such as water, alcohol (methanol and ethanol, etc.), and acetone can be used. Especially, for the pore forming material, a water-soluble compound is preferable and a water-soluble inorganic salt is more preferable. As the water-soluble inorganic salt, at least one selected from the group consisting of, for example, a sodium chloride, a potassium chloride, a magnesium chloride, a calcium chloride, a sodium silicate, a sodium carbonate, a sodium sulfate, a potassium sulfate, and a magnesium sulfate is preferable.

The average particle size of the pore forming material can be set, for example, in a range from 5 to 300  $\mu\text{m}$ . The size of the pores of the porous metal bonded grindstone obtained in accordance with the method for manufacturing the grindstone in the present invention corresponds to the size of the pore forming material. Therefore, the size of the formed pores can be adjusted by adjusting the particle size of the pore forming material. Further, the size of the pore forming material can be appropriately selected and used in consideration of the ease to remove it during the next step. If the average particle size of the pore forming material is too small, the vapor of the solvent is difficult to penetrate and the pore forming material is likely to remain in the molded body. Therefore, the lower limit of the average particle size is

preferably at least 5  $\mu\text{m}$  and may be at least 10  $\mu\text{m}$ , at least 50  $\mu\text{m}$ , or at least 80  $\mu\text{m}$ . Meanwhile, if the average particle size is too large, the number of the formed pores decreases, there occurs portions in which a bond matrix becomes large, and bond abrasion occurs in these portions, so that such abrasive grains become unsuitable for grinding high-hardness fragile materials. Therefore, the upper limit of the average particle size is preferably at most 250  $\mu\text{m}$  and may also be at most 200  $\mu\text{m}$  or at most 100  $\mu\text{m}$ .

10 The average particle size of the pores of the targeted porous metal bonded grindstone is appropriately selected depending on the size of the abrasive grains and the type of the material to be ground. In case of manufacturing the grindstone for grinding a silicon carbide (SiC) wafer using diamond abrasive grains having an average particle size of 8  $\mu\text{m}$ , the average particle size of the pore forming material is preferably from 70 to 200  $\mu\text{m}$ .

15 As described above, the average particle size of the pore forming material is the median size of the particle size distribution measured by a particle size distribution measuring instrument (laser refraction scattering method).

20 The porous metal bonded grindstone obtained in accordance with the method for manufacturing the grindstone in the present invention is a metal bond having pores. Therefore, the sharpness and the wear resistance are adjusted based on not a general degree of concentration, but based on the number of abrasive grains in a portion minus the pores from a grinding surface (so-called base portion). The abrasive grains, the metal powder, and the pore forming material 25 are preferably mixed such that the number of abrasive grains in the base portion minus the pores from the grinding surface is from 700 to 6500/cm<sup>2</sup>. If the number of abrasive grains in the base portion is too small, this leads to the porous metal bonded grindstone having a large amount of metal bonds per abrasive grain. Therefore, grain changeover of worn-away abrasive grains tend to be easily inhibited, so that this makes continuation of the processing difficult. If the number of abrasive grains in the base portion is too large, the weight 30 per abrasive grain tends to become low, so that the abrasive grains do not successfully eat into the high-hardness fragile material.

35 The number of abrasive grains in the base portion minus the pores from the grinding surface can be calculated based on the shape of the manufactured porous metal bonded grindstone as well as the mixture ratio of the abrasive grains, the metal powder, and the pore forming material. Further, in case of counting the number of abrasive grains from the obtained porous metal bonded grindstone, it can be determined by performing binarization in an image obtained by magnifying, by 500 times, the grinding surface minus the pores of the objective porous metal bonded grindstone and then counting the number of abrasive grains per unit area (cm<sup>2</sup>).

(Unfired Molded Body)

40 45 50 55 The unfired molded body is achieved by mixing the abrasive grains, the metal powder, and the pore forming material as well as filling and pressing (pressing at, for example, 500 to 5000 kg/cm<sup>2</sup>) the mixture in a predetermined molding die, thereby molding it into a predetermined shape.

60 The volume ratio (the volume of the pore forming material/the volume of the unfired molded body $\times 100\text{(\%)}$ ) of the pore forming material in the unfired molded body is preferably from 5 to 90 vol %. If the volume ratio of the pore forming material in the unfired molded body is smaller than 5 vol %, the grindstone would have a large number of metal bonds (would have a small number of pores). Therefore,

bond abrasion is likely to occur as in a grindstone without pores, and thus the grindstone would not be suitable for grinding high-hardness fragile materials. If the volume ratio is larger than 90 vol %, the grindstone would have a small number of metal bonds for holding the abrasive grains, so that it is difficult to maintain the structure.

The porosity of the pores of the obtained porous metal bonded grindstone corresponds to the amount of the pore forming material in the unfired molded body. Therefore, the porosity of the grindstone can be arbitrarily adjusted from a low porosity to a high porosity by adjusting the amount of the pore forming material. The volume ratio of the pore forming material in the unfired molded body is preferably at least 5 vol % and may be at least 10 vol %. Further, the volume ratio of the pore forming material in the unfired molded body is preferably at most 90 vol % and may be at most 85 vol %, at most 80 vol %, at most 75 vol %, at most 70 vol %, or at most 65 vol %.

Further, in order to realize the porous metal bonded grindstone having a low porosity which has been difficult to manufacture in accordance with the conventional manufacturing method, the volume ratio of the pore forming material in the unfired molded body may be in a range from 5 to 35 vol % or from 10 to 30 vol %.

[Solute Removing Step (P2)]

The solute removing step is a step for bringing the vapor of a solvent having solubility with respect to the pore forming material into contact with the unfired molded body to remove the pore forming material and to obtain the unfired molded body having pores. In the solute removing step, usually, the unfired molded body is taken out from a molding die and the unfired molded body is brought into contact with the vapor of the solvent for melting the pore forming material. In this manner, it becomes possible to efficiently remove the pore forming material in the unfired molded body and form the pores in the portion where the pore forming material had existed.

As the method for bringing the vapor of the solvent having solubility with respect to the pore forming material into contact with the unfired molded body, there is, for example, a method for supplying, to the unfired molded body, the vapor generated by heating a solvent at its boiling point or higher and a method for introducing the unfired molded body into a processing part filled with the vapor of a solvent. For example, in case of bringing water vapor into contact with the unfired molded body, the water vapor generated by a water vapor generator can be supplied to the unfired molded body and a humidifying furnace can be used. Further, in consideration of, for example, the type of the solvent to be used and the permeability of the vapor of the solvent into the unfired molded body, the contact may take place in a pressurized state and a depressurized state.

The solvent as the vapor brought into contact with the unfired molded body has only to be a solvent by which the pore forming material is melted (i.e., having solubility with respect to the pore forming material) and can be appropriately selected depending on the type of the pore forming material. In consideration of ease in handling and vaporizing etc., the vapor of a solvent containing at least one selected from the group consisting of water, alcohol, and acetone is preferably used. More preferably, the vapor of the solvent containing water is used.

The temperature of the vapor of the solvent is preferably at least the boiling point of the solvent to be used, is preferably at or below the firing temperature during the firing step, and is appropriately set depending on the type of

the solvent, etc. For example, in case of water vapor, the temperature can be set in a range from 100 to 200° C.

The time for bringing the vapor of the solvent into contact with the unfired molded body has only to be at least the time when the pore forming material can dissipate and is appropriately set depending on the type of the pore forming material and the ratio in the unfired molded body. For example, the time can be set to from 12 to 120 hours and from 24 to 72 hours.

[Firing Step (P3)]

The firing step is a step for firing the unfired molded body having pores. The firing step may be carried out by a publicly known method. For example, the unfired molded body having pores after the solute removing step is subjected to a heat processing in a firing furnace at a firing temperature preset in a range from 200° C. to 900° C. in a depressurized state or a normal pressure state, so that the metal powders are mutually melted and bonded while formed pores are in a state of being maintained, thereby forming the metal bond. In this manner, a porous fired body can be obtained.

[Porous Metal Bonded Grindstone]

The porous metal bonded grindstone obtained in accordance with the method for manufacturing the grindstone in the present invention is composed of the porous fired body. FIG. 2 is a partial cross sectional schematic drawing showing the porous metal bonded grindstone manufactured in accordance with the method for manufacturing the grindstone in the present invention. FIG. 3 is a drawing for explaining a state of the porous metal bonded grindstone at the time of grinding. As shown in FIGS. 2 and 3, a porous metal bonded grindstone 10 manufactured in accordance with the method for manufacturing the grindstone in the present invention contains a metal bond 12, abrasive grains 14, and pores 16.

The porous metal bonded grindstone 10 having the above structure has the following advantages.

As shown in FIG. 3, due to the porous structure, a contact area of the metal bond 12 in contact with a material 30 to be ground is reduced. In this manner, the bond abrasion can be alleviated and, at the same time, a contact surface pressure with respect to the material 30 to be ground can be increased. Pores 16 on a grinding surface 18 contributes as a chip pocket and is expected to improve performance of discharging chips 32 at the time of the grinding, while also improving a cooling function.

Further, in the structure of the porous metal bonded grindstone 10 are the pores 16 and therefore the strength of the porous metal bonded grindstone is lowered. Thus, an abrasive grain 14 whose lifetime is finished due to the grinding is made to fall and a self-sharpening effect for transferring the role to the next abrasive grain 14 works effectively, so that the successive grinding is possible with a stable load.

In the porous metal bonded grindstone 10, the pore diameter of the pores is from 5 to 300  $\mu\text{m}$ . The pore diameter of the pores may also be at least 10  $\mu\text{m}$ , at least 50  $\mu\text{m}$ , or at least 80  $\mu\text{m}$ . The pore diameter of the pores may also be at most 250  $\mu\text{m}$ , at most 200  $\mu\text{m}$ , or at most 100  $\mu\text{m}$ . The pore diameter can be controlled by adjusting the particle size of the pore forming material. The value of the pore diameter is determined by respectively measuring the average diameters of the long diameters and the short diameters of 50 pores as well as further calculating the average value of the 50 pores in ten 500 $\times$  magnified images of the grinding surface of the porous metal bonded grindstone.

Further, the porosity of the porous metal bonded grindstone **10** is from 5 to 90 vol %. The porosity of the porous metal bonded grindstone **10** may also be at least 10 vol %. Further, the porosity of the porous metal bonded grindstone **10** may also be at most 85 vol %, at most 80 vol %, at most 75 vol %, at most 70 vol %, or at most 65 vol %. The porosity can be controlled by adjusting the ratio of the pore forming material. The porosity is a value determined by calculating the density from the volume and the mass of the porous metal bonded grindstone as well as by calculating the calibration curve indicating the relationship between the predetermined density and the porosity (vol %).

As described above, according to the method for manufacturing the grindstone in the present invention, the porous metal bonded grindstone having a low porosity can be manufactured without using a closed-cell cellular material. For example, according to the method for manufacturing the grindstone in the present invention, it is also possible to manufacture a porous metal bonded grindstone which does not include a closed-cell cellular material such as hollow fine particles, is substantially composed of the metal bond **12**, the abrasive grains **14**, and pores **16** (namely, inclusion of inevitably contained impurities is not excluded), and has a low porosity such as 5 to 35 vol % or 10 to 30 vol %. Presence or absence of the closed-cell cellular material can be determined from, for example, analysis of a component of the contour of the pores.

On the grinding surface **18** of the porous metal bonded grindstone **10**, the number of abrasive grains in contact with the surface is from 700 to 6500/cm<sup>2</sup>. The number of abrasive grains can be controlled by adjusting the ratio of the abrasive grains, the metal powder, and the pore forming material. As described above, when the number of abrasive grains in contact with the surface is set in a range from 700 to 6500/cm<sup>2</sup>, the cut depth into the material to be ground composed of a high-hardness fragile material can be ensured, so that the abrasive grains become more suitable for grinding at low load even during high-speed feeding.

The shape of the porous metal bonded grindstone manufactured in accordance with the method for manufacturing the grindstone in the present invention is not particularly limited. A molding die used at the molding step (P1) is appropriately selected depending on the usage, to make it possible to obtain the porous metal bonded grindstone (fired body) assuming arbitrary shapes such as a plate type, a square pillar type, a circular type, a ring type, and an arc type.

#### <Method for Manufacturing Porous Metal Bonded Wheel>

FIG. 4 is a process chart of the method for manufacturing the porous metal bonded wheel in the present invention. As shown in FIG. 4, the porous metal bonded wheel having a base metal and the porous metal bonded grindstone bonded to the base metal can be obtained by the steps of: (P4) bonding, to a base metal, the porous metal bonded grindstone manufactured in accordance with the method for manufacturing the porous metal bonded grindstone in the present invention; and (P5) finishing the porous metal bonded grindstone bonded to the base metal by using a dresser.

FIG. 5 is a perspective view showing one example of the porous metal bonded wheel obtained in accordance with the method for manufacturing the porous metal bonded wheel in the present invention. A porous metal bonded wheel **100** has a disk-type base metal **20** made from metal such as iron and aluminum as well as segment chips **22**. The segment chip **22** is composed of the porous metal bonded grindstone **10**. The porous metal bonded grindstone **10** is manufactured in

accordance with the method for manufacturing the grindstone in the present invention. The base metal **20** is attached to a main shaft of a non-illustrated grinding machine, so that the porous metal bonded wheel **100** can be driven to rotate. The porous metal bonded wheel **100** has an outer diameter of about 250 mm and the segment chip **22** has a width of about 3 mm.

As shown in FIG. 5, a plurality of segment chips **22** are fixed annularly lined along an outer circumferential edge of a lower surface of the base material **20**. In the porous metal bonded wheel **100**, the segment chips **22** constitute an annular grinding surface **18**, which protrudes toward one surface side (in a direction parallel to a rotary shaft core (downward in FIG. 5)). Next, the segment chips **22** bonded to the base metal are finished by means of a dresser. In this manner, the porous metal bonded wheel **100** can be obtained.

Further, in the porous metal bonded wheel **100**, the segment chips **22** are composed of the porous metal bonded grindstones **10**, while the bonding may take place such that only the surface layers of the segment chips **22** are composed of the porous metal bonded grindstones **10**.

The porous metal bonded wheel **100** can be used for grinding high-hardness fragile materials such as a silicon carbide (SiC) wafer or a sapphire wafer. The porous metal bonded grindstone **10** of the porous metal bonded wheel **100** makes the grinding surface **18** slidably contact with the high-hardness fragile materials such as a silicon carbide (SiC) wafer or a sapphire wafer, accompanied by rotation of the base metal **20**, thereby grinding the high-hardness fragile materials into a flat type.

## EXAMPLES

Hereinafter, the present invention will be further explained in detail by way of examples. The present invention is not limited to the examples shown below as far as its gist is not changed.

#### [Example 1]: Manufacture of Test Piece of Porous Metal Bonded Grindstone

##### Materials

Abrasive grains: Diamonds (average particle size of 8 µm)

Metal powder (material which forms a metal bond): Mixture of Cu of 60 mass % and Sn of 40 mass %

Pore forming material: Sodium sulfate (average particle size of 70 µm)

##### Manufacturing Method

As shown in Table 1, a molding die is filled with a mixture of predetermined abrasive grains, metal powder, and pore forming material and subjected to pressure (500 to 5000 kg/cm<sup>2</sup>, room temperature), so that an unfired molded body was obtained.

Next, the unfired molded body was taken out from the molding die and was exposed to a water vapor atmosphere (100 to 200° C.) for 72 hours.

After exposed to the water vapor, the unfired molded body was fired (at 200 to 900° C.), so that the test piece (size: 40 mm in length×7 mm in width×4 mm in thickness) of the porous metal bonded grindstone was obtained.

TABLE 1

| (Abrasive grains + metal powder):pore forming material (Volume ratio) | The number of abrasive grains in the base portions (number of pieces/cm <sup>2</sup> ) | Porosity (vol %) | Pore diameter (μm) |
|-----------------------------------------------------------------------|----------------------------------------------------------------------------------------|------------------|--------------------|
| Example 1-1                                                           | 90:10                                                                                  | 700              | 10                 |
| Example 1-2                                                           | 70:30                                                                                  | 700              | 30                 |
| Example 1-3                                                           | 50:50                                                                                  | 700              | 50                 |
| Example 1-4                                                           | 10:90                                                                                  | 700              | 90                 |

The cross sections of the manufactured test pieces in Examples 1-1 to 1-4 were observed by using an SEM/EDS apparatus. As a result of performing EDS analysis on all the test piece cross sections, no residues of the pore forming material were observed and it could be confirmed that all the residues dissipated. Further, as a result of performing particle analysis by binarization of the SEM images (500 $\times$ ) of the test piece cross sections, all the test pieces indicate the same area ratio as the designed porosity and it could be confirmed that the porous metal bonded structure as designed was realized. Further, it could be confirmed that the pore diameter also corresponds to the average particle size of the pore forming material used.

#### Example 2

Except for changing the molding die, so that the size of the obtained porous metal bonded grindstone is 35 mm in length, 3 mm in width, and 9 mm in thickness, the porous metal bonded grindstone having the porosity in Table 2 was manufactured in the same manner as in Example 1.

The obtained porous metal bonded grindstones were bonded to the underside of the base metal having an outer diameter of 300 mm as shown in FIG. 5, so that the porous metal bonded wheel was manufactured.

The processing test for the high-hardness fragile material was performed by using the porous metal bonded wheel in Example 2 under the following grinding test conditions in order to evaluate the grinding resistance and the grindstone wear rate. The results are shown in Table 2.

The grinding resistance is a driving current value of the electric motor for driving and rotating the porous metal bonded grindstone during the grinding under the following grinding test conditions. Further, the grindstone wear rate is determined by indicating, as a rate, a wear amount of a grindstone sample in one grinding under the following grinding test conditions and by dividing a wear amount (thickness) of the grindstone by a machining allowance (thickness) of a workpiece. For example, if the grindstone wears by 100  $\mu$ m at the time of machining a wafer (workpiece) with a machining allowance by 50  $\mu$ m, the grindstone wear rate is 200%.

#### (Grinding Test Conditions)

Grinding machine: flat surface grinding machine (infeed system)

Grinding method: wet-type flat surface grinding

Workpiece: 4-inch single crystal silicon carbide (SiC) wafer

Machining conditions: the number of grindstone rotations of 2400 rpm, the number of wafer rotations of 400 rpm, cutting speed of 0.5  $\mu$ m/sec, and machining allowance of 200  $\mu$ m

Grinding fluid: Water-soluble grinding fluid

Comparative Example

The same as in Example 1 applied except for not using the pore forming material, so that the metal bonded grindstone having a porosity of 0 vol % was obtained. As in Example 2, the grinding test was performed by using the metal bonded wheel in which the obtained metal bonded grindstones are bonded to the base metal. The results are shown in Table 2.

TABLE 2

|                     | Porosity (vol %) | Grinding resistance (A) | Grindstone wear rate (%) |
|---------------------|------------------|-------------------------|--------------------------|
| Example 2-1         | 10               | 15.8                    | 0.70                     |
| Example 2-2         | 30               | 14.5                    | 3.80                     |
| Example 2-3         | 50               | 13.1                    | 24.50                    |
| Example 2-4         | 90               | 10.5                    | 113.90                   |
| Comparative example | 0                | Machining is impossible |                          |

It could be confirmed that, the higher the porosity was, the lower the machining resistance became and meanwhile, the wear amount tended to increase. It could also be confirmed that achieving a low porosity was effective for improving the wear resistance as a tool.

#### Example 3

The porous metal bonded grindstone was manufactured by using the pore forming material having the average particle size shown in Table 3, and was manufactured in the same manner as in Example 1 except for the porosity being 60 vol % and the number of abrasive grains being 700/cm<sup>2</sup>. As in Example 2, the grinding test was performed by using the porous metal bonded wheel in which the obtained porous metal bonded grindstones are bonded to the base metal. The results are shown in Table 3.

TABLE 3

|             | Average particle size of the pore forming material (μm) | Grinding resistance (A) | Grindstone wear rate (%) |
|-------------|---------------------------------------------------------|-------------------------|--------------------------|
| Example 3-1 | 5                                                       | 16.1                    | 52.6                     |
| Example 3-2 | 70                                                      | 12.9                    | 36.9                     |
| Example 3-3 | 120                                                     | 11.7                    | 11.3                     |
| Example 3-4 | 160                                                     | 11.2                    | 10.1                     |
| Example 3-5 | 250                                                     | 12.5                    | 5.7                      |
| Example 3-6 | 300                                                     | 15.3                    | 2.8                      |

#### Example 4

A porous metal bonded wheel was manufactured by bonding porous metal bonded grindstones having the number of abrasive grains in the base portions as shown in Table 4, a pore diameter of 70  $\mu$ m, and a porosity of 60 vol %. The grinding test was performed by using these grindstones. The results are shown in Table 4.

TABLE 4

|             | The number of abrasive grains in the base portions (number of pieces/cm <sup>2</sup> ) | Grinding resistance (A) | Grindstone wear rate (%) |
|-------------|----------------------------------------------------------------------------------------|-------------------------|--------------------------|
| Example 4-1 | 700                                                                                    | 12.9                    | 36.9                     |
| Example 4-2 | 1650                                                                                   | 13.2                    | 32.1                     |

## 13

TABLE 4-continued

|             | The number of abrasive grains in the base portions (number of pieces/cm <sup>2</sup> ) | Grinding resistance (A) | Grindstone wear rate (%) |   |
|-------------|----------------------------------------------------------------------------------------|-------------------------|--------------------------|---|
| Example 4-3 | 2300                                                                                   | 13.5                    | 24.8                     | 5 |
| Example 4-4 | 3650                                                                                   | 15.2                    | 16.6                     |   |
| Example 4-5 | 5800                                                                                   | 16.7                    | 13.8                     |   |
| Example 4-6 | 6500                                                                                   | 16.9                    | 13.1                     |   |

## INDUSTRIAL APPLICABILITY

The method for manufacturing the porous metal bonded grindstone in the present invention allows the grindstones having various porosities to be manufactured. The obtained grindstone and the porous metal bonded wheel comprising this grindstone can be used for grinding high-hardness fragile materials such as silicon carbide (SiC) wafer or sapphire wafer.

## REFERENCE SIGNS LIST

- 10 Porous metal bonded grindstone
- 12 Metal bond
- 14 Abrasive grains
- 16 Pore
- 18 Grinding surface
- 20 Base metal
- 22 Segment chip
- 30 Material to be ground
- 32 Chip
- 100 Porous metal bonded wheel

The invention claimed is:

1. A method for manufacturing a porous metal bonded grindstone, comprising:

## 14

a molding step for obtaining an unfired molded body including abrasive grains, metal powder and a pore forming material;

a solute removing step for bringing vapor of a solvent having solubility with respect to the pore forming material into contact with the unfired molded body to remove the pore forming material and to obtain an unfired molded body having pores; and  
a firing step for firing the unfired molded body having pores.

10 2. The method for manufacturing a porous metal bonded grindstone according to claim 1, wherein a volume ratio of the pore forming material to the unfired molded body is from 5 to 90 vol %.

15 3. The method for manufacturing a porous metal bonded grindstone according to claim 1, wherein an average particle size of the pore forming material is from 5 to 250  $\mu\text{m}$ .

4. The method for manufacturing a porous metal bonded grindstone according to claim 1, wherein the solvent contains at least one selected from the group consisting of water, 20 alcohol, and acetone.

5. The method for manufacturing a porous metal bonded grindstone according to claim 1, wherein the solvent contains water and

the pore forming material is a water-soluble compound.

25 6. The method for manufacturing a porous metal bonded grindstone according to claim 5, wherein the pore forming material is a water-soluble inorganic salt.

7. A method for manufacturing a porous metal bonded wheel, comprising the steps of:

30 bonding, to a base metal, a porous metal bonded grindstone manufactured in accordance with the method for manufacturing the porous metal bonded grindstone according to claim 1; and

finishing the porous metal bonded grindstone bonded to the base metal by using a dresser.

\* \* \* \* \*